

Oct. 16, 1928.

1,687,825

H. A. BRASSETT  
DIE BLOCK AND METHOD OF TREATING STEEL FOR  
USE IN THE MANUFACTURE THEREOF  
Filed Oct. 14, 1926

Fig. 1.



Fig. 2



Fig. 3.



Fig. 4.



Fig. 5.



Fig. 6.



Witness

Milton Lenoir

Inventor

Hermon A. Brassett,

By John L. Jamison.

Attorney

## UNITED STATES PATENT OFFICE.

HERMAN A. BRASSET, OF KENILWORTH, ILLINOIS.

## DIE BLOCK AND METHOD OF TREATING STEEL FOR USE IN THE MANUFACTURE THEREOF.

Application filed October 14, 1926. Serial No. 141,679.

My invention relates to the manufacture of die blocks and other special steel products requiring a steel which retains a high elastic limit in every direction under conditions of frequently repeated impact, and applies particularly to the mechanical refinement of the saine.

It is the usual practice to forge die blocks from an ingot cast of electric or open hearth alloy steel. Such ingots are either first rolled into blooms and then forged into billets under a forging press or hammer, or else they are immediately forged without rolling. In either case the pressure is applied to the sides of the ingot or bloom so as to elongate it and reduce its cross section, which produces a fibrous structure lengthwise or parallel with the longitudinal axis of the ingot.

It is a well known fact that the physical results obtained in testing steel are not the same in a test made parallel to the fibre as in one made transversely to the fibre. In the manufacture of die blocks it is customary, after the block has been suitably annealed, to make the die impressions in a surface of the block which is parallel with the fibre created by the elongation or reduction of the piece by rolling or forging. One reason for this has been that the center of an ingot shows a less dense structure than the outer layers, which is due to the more rapid cooling off and chilling of the rim which produces a closer structure therein, whereas the slow cooling of the center develops a coarser or less dense structure. The larger the ingot, the more pronounced is this condition and the more marked is the difference, but it is present in all ingots. This uneven density between surface and center is only partially counteracted in the process of reducing and by heat treatment which refines the grain but is not able to give a homogeneous structure from the surface to the center. The result is that the number of drop forgings obtainable from successive die sinkings, while satisfactory in the first few sinkings, becomes smaller as the center of the block is approached, is very unsatisfactory near the center, and increases again after the center is passed and the opposite surface approached. Since the resinking of dies is a very expensive operation, it can readily be understood that an important economy is to be gained by making the grain struc-

ture uniform throughout the block and equal in quality to that of the outer layers. While the desirability of such savings has long been recognized, prior to the present invention no satisfactory method has been proposed by which they could be realized.

I have found that I can overcome the lack of uniformity in the grain structure, and also produce a more compact grain structure throughout the block, by causing the blooms or billets which have been rolled or forged from the original ingot, and which, when necessary, have been cut into multiple pieces of approximately the weight of the finished die block, to be forged endwise or against the longitudinal fibre,—that is, in a direction perpendicular to that of the original forging or rolling, which is naturally in the direction of the length of the ingot. In the practice of my invention the endwise forging, or what is generally termed "upsetting", must be carried far enough so that the effect penetrates to the very center of the block. In other words, the center of the block must be subjected to the same mechanical refinement as the outer layers, as a slight upsetting of course does not materially affect the grain structure of the block, since it does not extend to any appreciable depth. That the desirable results referred to can be accomplished by my method, has been proven by physical tests of pieces of die blocks so forged, which show the same results as to ultimate strength, elastic limit, elongation, and reduction of area in their longitudinal and their transverse test pieces. It is well known that with the present method of forging the longitudinal tests are always superior to the transverse tests.

As a result of the uniform structure throughout the piece which I accomplish, I can with safety use one or the other of the faces at the upset ends for sinking the dies. This not only has the advantage that there is no reduction in the density of the structure reached in successive sinkings, but also the die impressions are cut across and not with the original fibre of the block, thereby obviating the yielding or flowing of the laminated fibrous structure under the great stress of impact and heat where the die impression is made in a longitudinal surface of the boom or billet.

In the use of my die block the continued impact of the drop forging hammer continues the refining action upon the block with the result that instead of deterioration from use 6 the grain structure of the block actually improves.

The accompanying drawings illustrate the several steps followed in practicing my improved process. Fig. 1 is a view of a steel 10 bloom or billet, the shade lines indicating the fibre running parallel with its longitudinal axis, and Fig. 2 is a cross-section thereof. Fig. 3 is a perspective view of a block cut from the billet shown in Fig. 1, illustrating 15 diagrammatically the old practice of sinking dies in the block parallel with the longitudinal fibres thereof. Fig. 4 is a view illustrating a billet cut to the weight required for a die block and arranged in position for forging, 20 as a step in my improved process. Fig. 5 is a view of the billet shown in Fig. 4 after it has been reduced by endwise forging or upsetting to the size required for a die block, and Fig. 6 is a view of the block shown in Fig. 25 5 with the die sunk in one of the upset ends of the block which are at right angles to the main axis of the original ingot. In all the views the shade lines are intended to represent the trend of the fibres. The views are 30 of course diagrammatic in character, but with the exception of Fig. 3 which shows the old practice as above stated, they serve to illustrate the several steps of my improved process.

35 In practicing my improved process I forge a billet 1 from the original ingot or rolled bloom in the usual manner, and cut the billet into multiples 2 of approximately the weight of the finished die block. These multiples 40 are forged under the press, including an endwise forging, against the longitudinal fiber resulting from the previous operations; in other words, the blocks are upset in this forging. For instance, a block of thirty inches 45 in height may be upset to one of only eighteen inches in height. The forging is done while the die block is hot, preferably at a temperature from 2000° to 2100° Fahrenheit, although the temperature may vary considerably 50 throughout a comparatively wide range, and after the forging has been done the block 3 is annealed in any suitable way. The die 4 is then cut into one end 5 of this block, facing the main axis of the original 55 ingot instead of being parallel with it as is the current practice as shown at 6 in the block 7 in Fig. 3. Forging in the manner described leaves the structure of the block 60 equally compressed throughout its entire mass, and in a refined state, incident to the work done on it while hot, so that the same character of grain structure of the metal is found in each successive sinking. The result 65 is a uniform life of the various sinkings,—that is to say, the number of forgings

made on each successive sinking is practically the same as on the first sinking, resulting in a much larger total number of forgings made from a given block.

In making die blocks according to the above described process I prefer to use a chrome-molybdenum-nickel steel so treated as to be suitable for use in making die blocks without being subjected to the usual or any treatment for hardening, because such a steel, besides 70 having the necessary strength, durability and toughness, is not too hard to be machined, or to be trimmed down for re-sinking after it has been used to such an extent that re-sinking is necessary or desirable, but my invention 75 may well be applied to die blocks made of steels that require hardening after the sinking of the die, and, therefore, it should be understood that the claims hereinafter made are not intended to be restricted to the use of 80 any particular alloy steel, or to the production of a die block material that essentially excludes hardening. Furthermore, it should be understood that my improved process may be applied in the treatment of high grade 85 steel for various other uses besides that of die block manufacture where a material of uniform grain structure throughout its mass is desired.

What I claim as my invention and desire 90 to secure by Letters Patent, is—

1. The method of making a die block and die from an elongated block having a longitudinal grain which consists in upsetting the block and foreshortening the same by forging 100 in the direction of the grain to substantially the finished dimensions and simultaneously refining the grain structure throughout the block, forming a die impression within the peripheral confines of a face transverse to the original longitudinal axis, and by the repeated impact of use, under a forging hammer further refining the remainder of the block. 105

2. A die block containing a die recess sunk into a face transverse to the original longitudinal axis of the billet from which the block is made and disposed within the peripheral confines of said face, said block having a grain refined by forging longitudinally of the original fibers and capable of further 110 refinement in use by repeated impact of the forging hammer in gaining impressions from the die. 115

3. A die block having a grain which has been refined throughout the entire length of the block by forging endwise of the original longitudinal fibers and having a forming die recess sunk into an end face thereof across the original trend of the fibers and within the peripheral confines of said end face. 120

4. A die block containing a forming die recess sunk into a face transverse to the original longitudinal axis of the billet from which the block is made, said block having a grain refined by forging longitudinally of the origi- 125

nal fibers and capable of further refinement in use by repeated impact of the forging hammer in gaining impressions from the die.

5. A body of metal suitable for use as a die block, comprising a block severed by a transverse cut from a billet which has a longitudinally extending grain, said block having a grain refined throughout by endwise forging

and being adapted thereby to have a forming die recess sunk in one end face thereof transverse to the original longitudinal grain, and being capable of further refinement in use by repeated impact of the forging hammer in gaining impressions from the die. <sup>10</sup>

HERMAN A. BRASSERT.